

## UNITED STATES PATENT OFFICE.

STERNER ST. P. MEEK, OF PHILADELPHIA, PENNSYLVANIA.

## TRACER COMPOSITION.

No Drawing.

Application filed May 21, 1924. Serial No. 714,919.

(GRANTED UNDER THE ACT OF MARCH 3, 1883, AS AMENDED APRIL 30, 1928; 370 O. G. 757.)

The invention described herein may be manufactured and used by or for the Government for governmental purposes without the payment to me of any royalty thereon.

The subject of this invention is a combustible composition or mixture burning with greater or less rapidity, as may be desired, and possessing the desirable quality of luminosity, brilliance or visibility in burning; the mixture being especially adapted for use as a tracer mixture in projectiles, though also useful in many other organizations, such as port fires, rockets, signal fires, and any burning composition in which the above mentioned qualities are desirable.

It has been found that the addition of certain rare earth elements to combustible materials will greatly increase luminosity, brilliance and visibility thereof when combustion takes place. These same elements, or proper salts thereof, when themselves combustible may be used either alone or in combination with other elements for the purpose above outlined.

While any rare earth elements possessing the characteristics, when heated, of giving off an unusually large proportion of its energy in the form of light waves, are adapted to produce the above outlined desired results; the preferred element for this purpose are zirconium and yttrium.

These elements may be used either in the form of nitrate or other oxygen carrier; in the form of a fuel, as sulpho-cyanate; or in the form of inert substances merely for increasing the brilliance, as an oxide or chloride.

The following tracer mixtures are typical examples of different association of these elements:

As an oxygen carrier:

|                     | Parts. |
|---------------------|--------|
| Magnesium           | 10     |
| Yttrium nitrate     | 15     |
| Zirconium nitrate   | 5      |
| Calcium resinate    | 5      |
| Lead sulpho-cyanate | 5      |
| Barium peroxide     | 10     |

| As an inert substance: |    | Parts. |
|------------------------|----|--------|
| Strontium nitrate      |    | 50     |
| Sodium nitrate         |    | 60     |
| Magnesium              |    | 40     |
| Calcium resinate       | 40 | 55     |
| Yttrium oxide          |    | 10     |
| Zirconium oxide        |    | 8      |

The following are typical examples of combustible mixtures of the elements:

|               |                   |
|---------------|-------------------|
| Zirconium     | 60 to 90 parts    |
| Yttrium       | 40 to 10 parts or |
| Yttrium salts | 60 to 90 parts.   |
| Zirconium     | 40 to 10 parts.   |

While the above mixtures are typical, they are cited only by way of example and are intended in no way to limit the proportions of the various ingredients to those set forth, as the proportions in which zirconium and yttrium will be used depend largely upon the other ingredients mixed therewith and the use to which the mixture is intended to be put.

What is claimed is:

1. A tracer composition for projectiles including an oxygen containing compound of an alkali earth metal, salts of a rare earth metal, a fuel and a binder.

2. A tracer composition for projectiles including an oxygen containing compound of an alkali earth metal, a sulphocyanate of a rare earth metal, an oxidizing agent and a binder.

3. A tracer composition for projectiles including as elements salts of yttrium and zirconium.

4. A tracer composition for projectiles including magnesium 10 parts, barium peroxide 10 parts, salts of yttrium and zirconium 20 parts, calcium resinate 5 parts and lead sulpho-cyanate 5 parts.

STERNER ST. P. MEEK.